

## UNITED STATES PATENT OFFICE.

LOUIS S. ROSS, OF NEWTONVILLE, MASSACHUSETTS.

## RAILWAY SIGNAL FUSEE, COMPOUND THEREFOR, AND METHOD OF MAKING SAME.

No Drawing.

Application filed April 30, 1920. Serial No. 377,940.

*To all whom it may concern:*

Be it known that I, LOUIS S. ROSS, a citizen of the United States, and a resident of Newtonville, in the county of Middlesex and 5 State of Massachusetts, have invented an Improvement in Railway Signal Fusees, Compounds Therefor, and Methods of Making Same, of which the following description is a specification.

10 This invention relates to railway signal fusees, igniting compounds therefor and the method of making the same.

In order that the principle of my invention may be readily understood, I have set 15 forth in the ensuing description one embodiment of the railway signal fusee and compound of my invention and the best mode known to me for igniting such fusee with my compound.

20 Railway signal fusees are preferably composed of potassium perchlorate, metallic nitrate, sulphur and carbonaceous material, or a hydrocarbon or a carbohydrate. For some years, such fusees have been manu-

25 factured containing potassium perchlorate instead of potassium chlorate with the result that accidental or spontaneous ignition fires resulting from railway signal fusees have been very largely, if not wholly, 30 eliminated. The color and brilliancy of the flame of the so-called perchlorate fusee are regarded as satisfactory but there is a general belief that such fusee does not have as good burning qualities as the so-called old

35 style sulphur and chlorate fusees. It has been attempted to overcome this objection by the addition of a small quantity of potassium chlorate to the potassium perchlorate mixture, and this is now permitted 40 by the bureau for the safe transportation of explosives and other dangerous articles provided the amount of potassium chlorate does not exceed 2.5% since this does not bring the temperature of ignition below 250° C.

45 It has heretofore been the practice to use either a match composition or some inflammable composition containing chlorate of potash and carbonaceous material that will ignite either by flame or with a com-

50 plementary material such as red phosphorus such composition being used as the so-called priming of the railway fusee. There is a comparatively low temperature incident to the combustion of the priming 55 in such case and while it has heretofore been the practice to use a potassium and sulphur

mixture together with metallic nitrates in the main burning composition of the fusee or compound therefor, the specifications of the said bureau for the safe transportation 60 of explosives, etc., require that "railway signal fusees shall not contain a mixture of chlorate and sulphur", and also require, as above stated, that the temperature of ignition of the composition must not be below 65 250° C.

In the manufacture of the said so-called perchlorate railway signal fusees considerable difficulty has been experienced in complying with such specifications in that the 70 fusees frequently fail to ignite in service, owing to the fact that the more stable potassium perchlorate has been substituted for potassium chlorate in the main burning portion or composition of the fusee. A potassium perchlorate composition has a very high 75 igniting point and in fact it is extremely difficult to ignite it with the flame of an ordinary match. In view of such difficulties in ignition, I have given very extensive 80 study to the problem and have, after an extensive period of experimentation, produced a new igniter or priming for fusees and like compositions with a consequent novel fusee, and have devised a new method 85 of ignition of fusees and compositions.

An important feature of my invention is the utilization of the reaction between an oxide, preferably a metallic oxide, and most desirably an iron oxide, and some substance 90 or substances capable of reducing or de-oxidizing the oxide and setting free molten metal, desirably iron, with generation of great heat.

Preferably I employ a magnetic iron oxide 95 and such oxide may be provided in iron spike or member or if desired I may employ iron filings or the so-called steel wool. Obviously, however, the desired metal may be utilized in any approved form. I do not 100 limit myself to the use of magnetic iron oxide as substantially the same result may be obtained, but not as rapidly or efficiently, if ordinary iron oxide be used instead. With such oxide or substance containing 105 oxide, I employ, as stated, some substance whereby the mixture may be ignited and the preliminary reaction started. Desirably also in the priming which contains such oxide I use some substance, preferably potassium chlorate, which when brought in contact with the striking member, results in 110

ignition that starts the reaction in the priming composition. Such striking member is desirably red phosphorus or a mixture of red phosphorus and antimony sulphide.

5 While I desire to claim broadly a compound, fusee or torch, and method, involving an oxide for the purpose stated, it is highly desirable that the priming be waterproof even when subjected to immersion in 10 water, owing to the conditions under which railway signal fusees must be used, and yet the priming must be capable of instant ignition and burning when the complementary material of the striking member is 15 brought into contact therewith.

In accordance with my invention, I effect the rapid and infallible ignition of perchlorate mixtures or compounds requiring a high mixing point, and in the practice of 20 my invention I bring molten metal, preferably iron, into close proximity to or into contact with the perchlorate mixture.

Heretofore in many cases the priming or chemical mixture has after ignition burned 25 itself out without communicating combustion to the main perchlorate composition, this being due to low combustion temperature, imperfect mixing of the chemicals or carelessness in applying the mixture. My 30 invention overcomes all these difficulties for in the practice thereof drops or particles of molten metal, such as iron, are brought into contact in a white hot state with the chemical compositions of the body of the fusee 35 requiring ignition. Once combustion is started in the priming of my invention, the rapidity of the chemical reaction reduces the iron or other oxide to a white incandescent mass, leaving small particles of molten 40 iron or other metal, desirably iron, in contact with the perchlorate or other composition and communicating flame thereto with rapidity and reliability.

To insure safety in mixing the materials 45 I desirably carefully mix the powdered chlorate of potassium magnetic iron oxide and other ingredients in a dry state, and then mix them with a liquid shellac containing the reducing material. This allows 50 the entire mixture to be poured into a small opening or depression in the compound of the railway fusee or torch. The alcohol in the shellac evaporates, and the priming thus 55 poured sets in a short time in a solid mass, and by the incorporation of the shellac mixture, there is furnished not only the necessary combustible material for the priming, but the desired imperviousness to moisture.

60 I have stated that the perchlorate fusee consists of potassium perchlorate, metallic nitrate, sulphur and a carbonaceous material. The said metallic nitrate is particularly susceptible to moisture, and it is there- 65 fore highly desirable that the opening in

the fusee leading to the body mixture or composition be sealed with a moisture resisting compound. This is effected in the practice of my invention.

Having thus set forth my invention I desire it to be understood that in practising the same many different formulas may be employed, and that I do not limit myself to any particular formula. I will, however, set forth a single formula from the use of 75 which I have obtained excellent results, without, however, limiting myself by so doing.

In accordance with such formula, I employ eighteen parts of chlorate of potassium, 80 one part of charcoal, two parts of umber, three-quarters of a part of strontium carbonate, and a sufficient quantity of liquid shellac (that is, shellac and alcohol). To three pounds of a mixture made up of the 85 foregoing ingredients in the proportions stated, I add one-half pound of magnetic iron oxide and one eighth of a pound of magnesium.

Chlorate of potassium and barium peroxide contain oxygen and the metals magnesium or aluminum have great affinity for oxygen, and when ignited they will so rapidly extract oxygen from mixtures containing these chemicals and containing 95 iron oxide or magnetic iron oxide ( $Fe_3O_4$ ) that the oxygen is rapidly extracted leaving the iron in a molten state and at such a high temperature that it instantly communicates the flame to the material to be ignited.

I may in the practice of my invention and in the provision of the priming, provide barium peroxide, magnesium and aluminum, and I may omit one or even two of the last three substances although the results are not as satisfactory as in the case where all three are used. Moreover my invention may be practised without the use of shellac or equivalent, and without the use of chlorate of potassium, but by the use 110 of chlorate of potash I am enabled to ignite the mixture by contact with complementary material containing red phosphorous. If the shellac be omitted, the mixture is not waterproof, but I may omit it within the 115 scope and purpose of my invention.

I believe that I am the first to provide a priming that can be satisfactorily used for igniting compositions requiring a high degree of ignition, and which in its desirable 120 form is a solid, waterproof, inflammable mixture capable of withstanding shock, abuse and rough handling and yet capable of quick ignition in wind and rain.

Having thus described one embodiment 125 of my invention and the best method known to me for practising my invention, I desire it to be understood that although specific terms are employed, they are used in a generic and descriptive sense and not for 130

purposes of limitation, the scope of the invention being set forth in the following claims.

Claims—

5. A railway signal fusee containing potassium perchlorate, metallic nitrate, sulphur and a carbonaceous material, and a priming therefor containing eighteen parts of chlorate of potassium, one part of charcoal, twelve parts of umber, three quarters of a part of strontium carbonate, liquid shellac together with magnetic iron oxide and magnesium. 35
10. A railway signal fusee containing potassium perchlorate, metallic nitrate, sulphur and a carbonaceous material, and a priming therefor having incorporated therein chlorate of potassium, charcoal, umber, strontium carbonate, magnetic iron oxide and magnesium. 40
15. A railway signal fusee containing potassium perchlorate, metallic nitrate, sulphur and a carbonaceous material, and a priming therefor having incorporated therein chlorate of potassium, charcoal, umber, strontium carbonate, magnetic iron oxide and magnesium. 45
20. A railway signal fusee containing potassium perchlorate, metallic nitrate, sulphur and a carbonaceous material, and a priming therefor having incorporated therein potassium chlorate, umber, iron oxide and magnesium. 50
25. A railway signal fusee containing potassium perchlorate, metallic nitrate, sulphur and a carbonaceous material, and a priming therefor having incorporated therein potassium chlorate, umber, iron oxide and magnesium. 55
30. A railway signal fusee containing potassium perchlorate, metallic nitrate, sulphur and a carbonaceous material, and a priming therefor having incorporated therein, potassium chlorate, iron oxide and magnesium.

5. A railway signal fusee containing potassium perchlorate, metallic nitrate and sulphur, and a priming therefor containing potassium chlorate, iron oxide and magnesium.

6. A railway signal fusee containing potassium perchlorate, metallic nitrate and sulphur, and a priming therefor containing potassium chlorate and iron oxide.

7. A railway signal fusee containing potassium perchlorate, metallic nitrate, sulphur and a carbonaceous material, and a priming therefor containing chlorate of potassium, magnesium, umber, strontium carbonate and magnetic iron oxide. 40

8. A railway signal fusee containing potassium perchlorate, metallic nitrate, sulphur and a carbonaceous material, and a priming therefor containing chlorate of potassium, charcoal, strontium carbonate, iron oxide, umber, magnesium and aluminum. 45

9. A railway signal fusee containing potassium perchlorate, metallic nitrate, sulphur and a carbonaceous material, and a priming therefor containing chlorate of potassium and iron oxide. 50

In testimony whereof, I have signed my name to this specification.

LOUIS S. ROSS.